

Sept. 22, 1925.

1,554,368

A. A. RACKOFF ET AL

PROCESS AND APPARATUS FOR MAKING STEEL

Filed March 1, 1923

FIG. 1



FIG. 2



FIG. 3



FIG. 4



INVENTORS

Adolph A. Rackoff  
James Louis Sharkey  
D. K. Totten Brown  
Attorneys

## UNITED STATES PATENT OFFICE.

ADOLPH A. RACKOFF, OF WILKINSBURG, PENNSYLVANIA, AND JAMES LOUIS SHARKEY, OF NEW YORK, N. Y.

## PROCESS AND APPARATUS FOR MAKING STEEL.

Application filed March 1, 1923. Serial No. 222,119.

*To all whom it may concern:*

Be it known that we, ADOLPH A. RACKOFF and JAMES LOUIS SHARKEY, citizens of the United States, and residents of Wilkinsburg and New York, respectively, in the counties of Allegheny and New York, respectively, and States of Pennsylvania and New York, respectively, have invented a new and useful Improvement in Processes and Apparatus for Making Steel; and we do hereby declare the following to be a full, clear, and exact description thereof.

Our invention relates to the handling of molten steel and other metals while the metal is being transferred to molds from open hearth or other metallurgical furnaces.

The object of our invention is to improve the quality of the metal by removing impurities therefrom through the combined action of mechanical agitation and sub-atmospheric pressure. The agitation is relied upon to bring solid and liquid slag impurities to the surface of the metal while it is passing from the furnace to the pouring ladle and the sub-atmospheric pressure is employed to extract certain gases which are present in solution in the molten metal.

To these ends, we provide a ladle adapted to receive metal from an open hearth furnace, or other metallurgical furnace, and to deliver the metal into molds. We also provide means for interposing obstructions or baffles in the path of the flowing metal in such a way as to cause the metal to be agitated before it falls into the ladle, and we place the ladle, and preferably the agitating channel, in a partial vacuum by means of a suitable suction pump. Other novel features of our invention include means for skimming slag from the metal on its way to the ladle, an arrangement of gates for directing the flow of the metal, and a removable vacuum cap for covering the ladle and the agitating channel.

Our present invention is an improvement over the system of handling molten metal described and claimed in the prior application of Adolph A. Rackoff, filed October 4, 1920, Serial No. 414,581, and we employ certain features of the said prior system in carrying out our present invention.

In the accompanying drawing, Fig. 1 is a vertical sectional view showing somewhat diagrammatically a set of apparatus constructed in accordance with our invention,

the section being taken substantially on the line 1-1, Fig. 2; Fig. 2 is a plan view of the same apparatus; Fig. 3 is another vertical sectional view taken substantially on the line 3-3, Fig. 2; and Fig. 4 is a plan view of the same apparatus with the vacuum cap removed.

In the drawing, the numeral 2 indicates a portion of an open hearth steel furnace having a tapping notch 3 which discharges the molten metal into a runway 4 leading to a ladle device, with which our invention is particularly concerned. This device includes a body portion 5 which may be of any construction usual in ladles for handling metal, 70 and which may have in its bottom a pouring opening 6 controlled by a plug 7. Trunnions 8 are provided for lifting and transporting the ladle.

The top of the ladle 5 is covered by a member 9 which carries the agitating, skimming and flow-controlling arrangements, and above the member 9 is a vacuum cap 10 which is so shaped as to form a substantially gas-tight cover. The joints between the ladle 5, the member 9 and the cap 10 may be luted with clay or the like.

The member 9 is provided with a straight channel 11 communicating with the runway 4 and with a circularly curved channel 12 which receives the molten metal from the straight channel 11 and conveys it in a generally circular path to an opening 13 through which the metal falls into the body of the ladle 5. Baffles 14 extend into the channel 12 and cause the molten metal to move in a zig-zag path which agitates the metal and brings the slag to the surface. Beyond the baffles 14 the channel 12 is deepened, as shown at 15, to form a settling and storing receptacle 95 which receives the metal temporarily before it enters the body of the ladle.

We provide means for removing slag from the molten metal at two points during its passage through the channels described above. One of these slag-removing means consists of a chute 16 communicating with the straight channel 11 at a point above the bottom thereof, and the other consists of a spout 17 leading off from the curved channel 12 beyond the baffles 14 and from a point above the bottom thereof. Both the chute 16 and the spout 17 may discharge into a vertical chute 18 which conducts the slag into a slag car, not shown.

Various gates are provided for controlling the flow of metal and slag in the above described paths. A gate 20 is provided near the inlet end of the straight channel 11 for entirely shutting off the inlet to the ladle. A gate 21 controls communication between the channel 11 and the slag chute 16. A gate 22 controls the passage of metal from the straight channel 11 into the curved channel 12. A gate 23 controls the flow from the channel 12 into the slag spout 17, and a gate 24 controls the flow of metal from the reservoir 15 into the body of the ladle. All of these gates are composed of refractory material and slide in refractory guideways carried by the cover member 9. The gates may be raised and lowered by any ordinary means, which it is not considered necessary to illustrate in detail, since such arrangements are common in the art.

Pipes 26, 27 and 28 extend through the top of the vacuum cap 10, and all communicate with a horizontal pipe 29 which is connected to a suitable vacuum pump, not shown. The pipes 26 and 27 communicate with the space between the cap 10 and the cover member 9, while the pipe 28 extends through the cover member and communicates with the space in the body of the ladle. It will be evident that various other arrangements of pipes may be employed to place the interior of the apparatus under reduced pressure. For example, one or more suction pipes may be inserted through the side walls of the ladle 5 instead of inserting the pipe 28 into the ladle from above, as shown.

In the operation of handling metal by the use of the apparatus described above, the ladle is connected to the furnace in the manner shown, with the gates 20 and 22 open and the gate 21 closed. The metal which first flows from the furnace is thus caused to flow through the curved channel 12 around the baffles 14 which agitate the metal and cause any slag which may be contained within the body of the metal to rise to the surface, where it remains since it is lighter than the metal and is not subjected to any pressure tending to submerge it again. Such slag may be skimmed off through the slag spout 17, the entrance to which is located near the top of the stream of molten metal, and the gate 23 being raised sufficiently for this purpose. The metal then passes into the depression or reservoir 15 where it may be allowed to accumulate by closing the gate 24, or, if desired, the gate 24 may be kept open and the metal allowed to flow continuously through the opening 13 into the body of the ladle.

When slag begins to flow from the furnace the gate 21 is opened and the gate 22 is closed. The slag, which is on the surface of the stream of metal is thus deflected into

the slag chute 16 and passes to the slag car. Throughout the operation, the ladle is preferably kept under reduced pressure by operating the vacuum pump to which the pipe 29 is connected. The gate 20 is sealed by the metal flowing beneath it, and if the slag gate 23 is opened it is preferably opened only far enough to permit the slag to escape without permitting air to enter to a substantial extent. After the charge has been tapped from the furnace the gate 20 may be closed and the vacuum is maintained within the ladle as long as may be required, depending upon the degree of purification desired and the time required for pouring the metal into molds.

The system described above produces metal that is thoroughly cleansed, both by the removal of slag and by the extraction of some or all of the dissolved gases.

It will be understood that the foregoing details of construction are shown and described herein merely for the purpose of illustrating our invention, and that our invention is by no means limited to this particular structure, but may be carried out by means of any other apparatus and with any variations in the steps of the process such as fall within the scope of the appended claims.

We claim as our invention:

1. Metallurgical apparatus comprising a furnace, a container, means for conducting molten metal from said furnace to said container, means for withdrawing slag impurities from the molten metal while passing from the said furnace to the said container, and means for subjecting said metal to sub-atmospheric pressure while passing from said furnace to said container.

2. Apparatus for making steel comprising a ladle, means for causing molten metal to flow horizontally toward the said ladle and then to drop vertically into the said ladle, means for withdrawing slag impurities from the said metal while flowing toward said ladle, and means for maintaining said purifying means under sub-atmospheric pressure.

3. Apparatus for making steel comprising a ladle, means for causing molten metal to flow in an indirect path and thence into the said ladle, baffles extending into the path of the flowing metal from the sides thereof and adapted to remove impurities from the said metal, and means for maintaining said flow-directing and purifying means under sub-atmospheric pressure.

4. Apparatus for making steel comprising a ladle, means for causing molten metal to flow in an indirect path and thence into the said ladle, baffles extending into the path of the flowing metal from the sides thereof and adapted to remove impurities from the said metal, and means for main-

taining said flow-directing and purifying means under sub-atmospheric pressure and for also maintaining said ladle under sub-atmospheric pressure.

5. Apparatus for making steel comprising a ladle, a cover therefor having a channel for directing molten metal around the said ladle and then permitting the metal to drop vertically into said ladle, and means for maintaining said cover and said ladle under sub-atmospheric pressure.

6. Apparatus for handling molten metal comprising a ladle, a cover for the said ladle, said cover being provided with an annular channel for conducting molten metal, a cap above said cover, and means for exhausting air from the interior of said cap and from the interior of said ladle.

7. Apparatus for handling molten metal comprising a ladle, a cover for the said ladle, said cover being provided with an annular channel for conducting molten metal, a cap above said cover, means for exhausting air and gases from the interior of said cap and from the interior of said ladle, and baffles extending into said channel from opposite sides thereof.

8. Apparatus for handling molten metal comprising a ladle, a cover therefor provided with an annular channel having portions 30 of successively increasing depth, the portion of greatest depth communicating with an opening leading into the interior of said ladle, means for conducting slag from said metal, gates for controlling the flow of 35 molten material through said channel and through said slag-removing means, a cap above the said ladle and cover, and pipes extending through the said cap for maintaining the interior of the apparatus under 40 sub-atmospheric pressure.

9. The process of making steel which comprises melting a charge in a furnace, conducting said molten charge from said furnace in the form of a stream, agitating 45 said stream under sub-atmospheric pressure, and diverting the top portion of said stream to separate the slag contained therein from the main body of the stream.

In testimony whereof we the said ADOLPH 50 A. RACKOFF and JAMES LOUIS SHARKEY, have hereunto set our hands.

ADOLPH A. RACKOFF.  
JAMES LOUIS SHARKEY.